

## 1

3,038,798

### TITANIUM-NIOBIUM ALLOYS

Lewis W. Berger, Mayfield Heights, and Robert I. Jaffee and Dean N. Williams, Columbus, Ohio, assignors, by mesne assignments, to Kennecott Copper Corporation, New York, N.Y., a corporation of New York  
No Drawing. Filed May 2, 1960, Ser. No. 25,891  
3 Claims. (Cl. 75—174)

This invention relates to titanium-niobium-base alloys, particularly titanium rich and intermediate alloys containing up to 70 percent niobium.

This application is a continuation-in-part of our application Serial No. 575,937, filed April 4, 1956, now abandoned.

The binary titanium-niobium equilibrium diagram shows a beta-isomorphous system with a limited solubility of niobium in alpha titanium and a rather extensive alpha-beta field. At 1100° F., about 3 percent niobium can be dissolved in alpha, while the alpha-beta field extends from about 3 to 35 percent niobium. On quenching from the beta field, beta is completely retained at 36 percent niobium and above. The addition of a third element to Ti—Nb-base compositions provides further useful alloys.

It is an objective of this invention, therefore, to provide new and valuable titanium-niobium-base ternary alloys.

Still another object of this invention is to provide ternary alloys of titanium and niobium, and of titanium-niobium-base compositions, whereby valuable properties

## 2

base ternary alloys containing up to 70 percent niobium, up to 45 percent of an alloying addition, balance titanium. Specific alloying elements of interest include vanadium, tantalum, and zirconium.

Binary alloys of titanium and niobium have been prepared by melting in an inert tungsten-electrode arc furnace under a static argon partial pressure of 15 to 20 centimeters of mercury. Alloy compositions of 1.5 percent, 3 percent, 10 percent, 15 percent, 20 percent, 25 percent, 30 percent, 35 percent, 40 percent, 50 percent, 60 percent, and 70 percent niobium, balance essentially all titanium have been prepared. Except for some spattering during the melting of the 60 percent and 70 percent niobium alloys, no difficulties have been encountered in preparing these compositions. Alloy specimens containing up to 70 percent niobium have been forged in air to a  $\frac{3}{8}$ -inch-square cross section. The forged ingots have been rolled in air at 1500° F. to approximately 0.040-inch sheet, using 10 percent reduction per pass. The alloys may then be given an annealing or stabilizing treatment.

Ternary titanium-niobium-base alloys have also been prepared by melting in an inert tungsten-electrode arc furnace under a static argon partial pressure of 15 to 20 centimeters. Table I lists mechanical properties of some ternary alpha-beta-type alloys. Data for binary Ti—10Nb and Ti—15Nb compositions are included for comparison. The worked ternary alloys were all in the equilibrated-and-stabilized condition, i.e., held  $\frac{1}{2}$  hour at 1300° F., furnace cooled to 1100° F., held 1 hour and air-cooled.

Table I.—Mechanical Properties of Ti—Nb-Base Ternary Alpha-Beta Alloys

| Composition<br>Weight percent<br>(balance Ti) | Vickers hardness<br>Number 10-kg. load |         | Tensile<br>strength<br>(p.s.i.) | Yield strength, p.s.i. |             | Elongation, per-<br>cent in 1-inch |       | Reduction in<br>area,<br>percent | Bend<br>duc-<br>tility |  |
|-----------------------------------------------|----------------------------------------|---------|---------------------------------|------------------------|-------------|------------------------------------|-------|----------------------------------|------------------------|--|
|                                               | As-cast                                | Wrought |                                 | 0.1% offset            | 0.2% offset | Uniform                            | Total |                                  |                        |  |
|                                               |                                        |         |                                 |                        |             |                                    |       |                                  |                        |  |
| 10 Nb-----                                    | 205                                    | 191     | 71,000                          | 54,000                 | 58,000      | 10                                 | 18    | 47                               | 0                      |  |
| 15 Nb-----                                    | 242                                    | 197     | 74,000                          | 54,000                 | 60,000      | 8                                  | 13    | 33                               | 0                      |  |
| 10 Nb-5 V-----                                | 299                                    | 228     | 88,000                          | 77,000                 | 81,000      | 5                                  | 7     | 26                               | 0                      |  |
| 10 Nb-5 Ta-----                               | 233                                    | 207     | 81,000                          | 65,000                 | 70,000      | 6                                  | 10    | 32                               | 0                      |  |
| 10 Nb-5 Zr-----                               | 230                                    | 215     | 98,000                          | 77,000                 | 82,000      | 5                                  | 10    | 23                               | 0.5                    |  |

of heat-treatability and useful strength-ductility relationships may be obtained and/or combined.

Yet another object of this invention is to provide effective titanium-niobium-base ternary compositions, with tantalum, zirconium, or vanadium as the third component.

Other objects and advantages of the present invention will be apparent from the following examples and detailed descriptions thereof.

In general, this invention relates to titanium-niobium-

55 An investigation of the aging properties of the alpha-beta alloys has shown that alloys containing 10 percent niobium and 5 percent of another beta-stabilizing element have very high aging responses. In this investigation the ternary alpha-beta alloys were quenched from 1250° F. and 1550° F. and then aged at 800° F. for periods of time up to 16 hours. Alloys containing vanadium harden appreciably on quenching from either 1250° F. or 1550° F. Table II below shows the results of the aging studies in terms of hardness.

Table II.—Aging Response of Ternary Ti—Nb-Base Alpha-Beta Alloys Aged at 800° F.

| Alloy weight percent addition | Aging time, hours | Quench                   |                          |
|-------------------------------|-------------------|--------------------------|--------------------------|
|                               |                   | VHN(10-kg.) <sup>a</sup> | VHN(10-kg.) <sup>b</sup> |
| Ti-10 Nb-5 V                  | 0                 | 317                      | 239                      |
|                               | 1/4               | 333                      | 262                      |
|                               | 1                 | 317                      | 306                      |
|                               | 2                 | 309                      | 333                      |
|                               | 4                 | 319                      | 319                      |
|                               | 16                | 260                      | 354                      |
| Ti-10 Nb-5 Ta                 | 0                 | 236                      | 215                      |
|                               | 1/4               | 254                      | 210                      |
|                               | 1                 | 260                      | 215                      |
|                               | 2                 | 245                      | 225                      |
|                               | 4                 | 234                      | 247                      |
|                               | 16                | 235                      | 228                      |
| Ti-10 Nb-5 Zr                 | 0                 | 240                      | 240                      |
|                               | 1/4               | 251                      | 249                      |
|                               | 1                 | 242                      | 276                      |
|                               | 2                 | 233                      | 236                      |
|                               | 4                 | 242                      | 249                      |
|                               | 16                | 230                      | 260                      |

<sup>a</sup> Specimens held at 1,250° F. for 4 hours and water quenched prior to aging.

<sup>b</sup> Specimens held at 1,550° F. for 1 hour and water quenched prior to aging.

These investigations indicate the value of alpha-beta-type alloys containing from about 3 percent to about 30 percent niobium, from about 1 percent to about 10 percent of at least one of the alloying elements zirconium, tantalum, vanadium, balance essentially titanium. The data illustrate the useful properties of this alloy system.

In addition to the alpha-beta-type alloys discussed above, it has been found that titanium-niobium-base ternary alloys of the beta type possess valuable properties and useful characteristics. Table III below lists the mechanical properties of these Ti—Nb-base ternary alloys.

they do at the lower temperatures. Thus, they provide useful high temperature alloys. Additions of from about 5 percent to about 45 percent of the elements to titanium-niobium alloys containing 30 to 70 percent niobium are beneficial. Outstanding hot hardness properties are obtained by adding 30 to 40 percent of vanadium or zirconium to titanium-niobium alloys containing about 40 to 60 percent niobium.

Other alloy systems disclosed possess extremely valuable properties. For example Ti—50Nb-base alloys containing vanadium and zirconium have excellent room-temperature ductility, very good uniform elongation, and improved strength at 1650° F. It is clear also that complex alloys containing combinations of the individual alloying elements will possess equally important and worthwhile properties.

Table IV.—Hot Hardness of Ti—Nb Base Alloys

|    | Composition, weight percent (balance Ti) | Hardness, <sup>a</sup> DPH, kg./mm. <sup>2</sup> , at temperature ° F. indicated |     |       |       |
|----|------------------------------------------|----------------------------------------------------------------------------------|-----|-------|-------|
|    |                                          | 75                                                                               | 930 | 1,290 | 1,650 |
| 25 | 50 Nb                                    | 138                                                                              | 94  | 40    | 19    |
|    | 60 Nb                                    | 146                                                                              | 107 | 66    | 40    |
|    | 70 Nb                                    | 159                                                                              | 96  | 79    | 58    |
|    | 50 Nb-5 V                                | 164                                                                              | 177 | 78    | 37    |
|    | 50 Nb-10 B                               | 199                                                                              | 162 | 100   | 42    |
|    | 50 Nb-20 V                               | 272                                                                              | 217 | 139   | 74    |
|    | 50 Nb-30 V                               | 283                                                                              | 229 | 194   | 141   |
|    | 50 Nb-40 V                               | 304                                                                              | 282 | 242   | 178   |
| 30 | 50 Nb-5 Ta                               | 140                                                                              | 83  | 46    | 25    |
|    | 50 Nb-10 Ta                              | 149                                                                              | 87  | 52    | 27    |
|    | 50 Nb-20 Ta                              | 179                                                                              | 152 | 113   | 99    |
|    | 50 Nb-10 Zr                              | 167                                                                              | 149 | 89    | 47    |
|    | 50 Nb-20 Zr                              | 209                                                                              | 179 | 119   | 70    |
|    | 50 Nb-30 Zr                              | 249                                                                              | 198 | 149   | 121   |

<sup>a</sup> Elevated-temperature tests were conducted in a vacuum of less than 5 microns, using a load of 730 grams and an indentation time of 10 seconds

Table III.—Mechanical Properties of Ti—Nb-Base Ternary Beta Alloys

| Composition weight percent (balance Ti) | Vickers hardness number 10-kg. load |                      | Tensile strength (p.s.i.) | Yield strength, p.s.i. |         | Elongation, percent in 1 inch |    | Reduction in area, percent | Bend ductility |  |  |  |
|-----------------------------------------|-------------------------------------|----------------------|---------------------------|------------------------|---------|-------------------------------|----|----------------------------|----------------|--|--|--|
|                                         | As-cast                             | Wrought <sup>a</sup> |                           | 0.1% Offset            |         | 0.2% Offset                   |    |                            |                |  |  |  |
|                                         |                                     |                      |                           |                        |         |                               |    |                            |                |  |  |  |
| 50 Nb                                   | 153                                 | 138                  | 58,000                    | 58,000                 | 58,000  | 0                             | 0  | 51                         | 0              |  |  |  |
| 50 Nb-5 V                               | 161                                 | 164                  | 72,000                    | 72,000                 | 72,000  | 10                            | 17 | 47                         | 0              |  |  |  |
| 50 Nb-10 V                              | 219                                 | 199                  | 83,000                    | 80,000                 | 80,000  | 13                            | 18 | 42                         | 0              |  |  |  |
| 50 Nb-20 V                              | 266                                 | 272                  | 106,000                   | 98,000                 | 98,000  | 13                            | 18 | 40                         | 0              |  |  |  |
| 50 Nb-30 V                              | 249                                 | 283                  | 126,000                   | 118,000                | 119,000 | 13                            | 17 | 48                         | 0              |  |  |  |
| 50 Nb-40 V                              | 285                                 | 304                  | 141,000                   | 134,000                | 135,000 | 3                             | 3  | 8                          | 1.0            |  |  |  |
| 50 Nb-50 V                              | 360                                 | 390                  |                           |                        |         |                               |    |                            |                |  |  |  |
| 50 Nb-5 Ta                              | 177                                 | 140                  | 63,000                    | 63,000                 | 63,000  | 0                             | 16 | 41                         | 0              |  |  |  |
| 50 Nb-10 Ta                             | 181                                 | 149                  | 66,000                    | 65,000                 | 66,000  | 0                             | 16 | 54                         | 0              |  |  |  |
| 50 Nb-20 Ta                             | 202                                 | 179                  | 74,000                    | 74,000                 | 74,000  | 12                            | 19 | 54                         | 0              |  |  |  |
| 50 Nb-30 Ta                             | 207                                 | 206                  |                           |                        |         |                               |    |                            |                |  |  |  |
| 50 Nb-40 Ta                             | 206                                 | 224                  |                           |                        |         |                               |    |                            |                |  |  |  |
| 50 Nb-50 Ta                             | 169                                 | 233                  |                           |                        |         |                               |    |                            |                |  |  |  |
| 50 Nb-10 Zr                             | 215                                 | 167                  | 780,000                   | 77,000                 | 77,000  | 8                             | 13 | 39                         | 0              |  |  |  |
| 50 Nb-20 Zr                             | 245                                 | 209                  | 100,000                   | 95,000                 | 96,000  | 9                             | 13 | 40                         | 0              |  |  |  |
| 50 Nb-30 Zr                             | 262                                 | 249                  | 114,000                   | 110,000                | 110,000 | 13                            | 20 | 55                         | 0              |  |  |  |
| 50 Nb-40 Zr                             | 268                                 | 276                  |                           |                        |         |                               |    |                            |                |  |  |  |
| 50 Nb-50 Zr                             | 272                                 | 272                  |                           |                        |         |                               |    |                            |                |  |  |  |

<sup>a</sup> Samples held 2 hours at 1,450° F. and water quenched.

Mechanical-property data for the Ti—50Nb binary composition are included in the table for purposes of comparison. It should be noted that the ternary additions strengthened the base material. These alloys also show considerable increase in uniform elongation over the binary 50 percent niobium composition.

Hot-hardness data for the alloys are presented in Table IV. Values are tabulated for 75° F., 930° F., 1290° F., and 1650° F.

At 930° F. and 1290° F. vanadium gives the most effective strengthening per unit ternary addition, followed in order by zirconium and tantalum. However at 1650° F. the order is zirconium, vanadium and tantalum. At 20 percent addition and above, the ternary additions vanadium, zirconium, and tantalum strengthen much more, proportionately, at the higher temperatures than

the data in Table V below show the results of tests to determine the resistance of the Ti—Nb base ternary alloys to oxidation in a static atmosphere at elevated temperatures. Specimens used in obtaining these data were about 0.25 x 0.50 x 0.04 inch and were prepared as follows:

Each specimen was carefully finished on 400-grit paper, cleaned in a solvent, weighed and measured. Each specimen was then placed on a small ceramic ring and set inside a crucible cover. A second, larger ceramic ring was then placed around each specimen to insure retention of any spattered scale.

Each specimen assembly, prepared as described above, was placed on a firebrick and, thus supported, inserted into a furnace which had been brought up to the test temperature. The specimens were in this manner exposed to air oxidation for periods of 16 hours at test tem-

peratures of 1400° F. and 1800° F. After exposure for the prescribed time, the treated specimens were covered with a second crucible cover and cooled. In this way, the loss of oxidation products during the cooling period was avoided.

After the specimens had been cooled, they were each weighed to determine the weight gain of each specimen. From this, the weight increase per unit original area was computed for each specimen. The samples were then brushed with a wire brush to remove loose scale, and the percentage of original sample remaining was then determined. In many cases the scale proved to be tightly adherent and could not be removed entirely, which accounts for the fact that values greater than 100 are reported in several instances under "percent of original sample remaining." The samples were then sectioned centrally, mounted in Bakelite, polished, and etched for microexamination. The thickness of unaffected base material was measured by means of a calibrated movable stage. Finally, hardness readings were taken in the center of the cross section. Values obtained in accordance with the procedures described above were as follows:

Table V.—Resistance of Ti—Nb Base Alloys to Oxidation in a Static Atmosphere

| Composition weight percent (balance Ti) | Original Vickers hardness (10-kg. load) | 16 hours at 1,400° F.                               |                                           |                                      |                                | 16 hours at 1,800° F.                               |                                           |                                      |                                |
|-----------------------------------------|-----------------------------------------|-----------------------------------------------------|-------------------------------------------|--------------------------------------|--------------------------------|-----------------------------------------------------|-------------------------------------------|--------------------------------------|--------------------------------|
|                                         |                                         | Weight increase per unit original area, mg./sq. cm. | Penetration of contaminant per side, inch | Percent of original sample remaining | Vickers hardness (10-kg. load) | Weight increase per unit original area, mg./sq. cm. | Penetration of contaminant per side, inch | Percent of original sample remaining | Vickers hardness (10-kg. load) |
| 50 Nb.....                              | 138                                     | 2.58                                                | 0.0063                                    | 101                                  | 202                            | 73.7                                                | Total                                     | 18                                   | 370                            |
| 60 Nb.....                              | 146                                     | 3.54                                                | 0.0063                                    | 101                                  | 155                            | 61.5                                                | Total                                     | 46                                   | 380                            |
| 70 Nb.....                              | 159                                     | 6.96                                                | 0.0052                                    | 97                                   | 156                            | 92.4                                                | Total                                     | 16                                   | -----                          |
| 50 Nb-5 V.....                          | 164                                     | 3.90                                                | 0.0065                                    | 101                                  | 180                            | 52.9                                                | Total                                     | 0                                    | -----                          |
| 50 Nb-10 V.....                         | 199                                     | 7.20                                                | 0.0057                                    | 103                                  | 215                            | 72.6                                                | Total                                     | 0                                    | -----                          |
| 50 Nb-20 V.....                         | 272                                     | 14.17                                               | 0.0040                                    | 103                                  | 238                            | 126.9                                               | Total                                     | 0                                    | -----                          |
| 50 Nb-30 V.....                         | 283                                     | 172.6                                               | Total                                     | 0                                    | 171.0                          | Total                                               | 0                                         | -----                                | -----                          |
| 50 Nb-40 V.....                         | 304                                     | 108.4                                               | Total                                     | 0                                    | 108.5                          | Total                                               | 0                                         | -----                                | -----                          |
| 50 Nb-5 Ta.....                         | 140                                     | 2.86                                                | 0.0063                                    | 101                                  | 210                            | 63.4                                                | Total                                     | 37                                   | 376                            |
| 50 Nb-10 Ta.....                        | 149                                     | 3.25                                                | 0.0060                                    | 101                                  | 170                            | 62.6                                                | Total                                     | 57                                   | 409                            |
| 50 Nb-20 Ta.....                        | 179                                     | 4.67                                                | 0.0040                                    | 101                                  | 170                            | 65.2                                                | Total                                     | 29                                   | 380                            |
| 50 Nb-10 Zr.....                        | 167                                     | 4.31                                                | 0.0033                                    | 102                                  | 357                            | 72.0                                                | Total                                     | 10                                   | -----                          |
| 50 Nb-20 Zr.....                        | 209                                     | 17.44                                               | 0.0068                                    | 98                                   | 276                            | 69.9                                                | Total                                     | 0                                    | -----                          |
| 50 Nb-30 Zr.....                        | 249                                     | 112.1                                               | Total                                     | 0                                    | 73.0                           | Total                                               | 0                                         | -----                                | -----                          |

From the values listed above it is apparent that 16 hours' exposure at 1400° F. had no unduly severe effects on most of the alloys. Except for the Ti—50 Nb—20 Zr alloy, which flaked slightly, a tightly adherent scale was formed on all the specimens. As has been noted above, this scale could not always be entirely removed by a wire brush, and consequently many of the values for "percent of original sample remaining" are in excess of 100.

The alloys of this invention will find many applications. They are particularly useful for structural members for high temperature applications. They are useful for mis-

siles, for jet engine parts and for such specific uses as leading edge wing sections of high speed aircraft for upper atmosphere operation.

5 New and useful alloys of titanium and niobium and of titanium-niobium-base alloys having been described and characterized, it is desired to further define the invention according to the following claims.

What is claimed is:

1. Titanium-niobium alloys consisting of from about 40 percent to about 60 percent niobium, from about 30 percent to about 40 percent vanadium, balance titanium, said alloys being characterized by good hot hardness properties.
2. Titanium-niobium alloys consisting of from about 40 percent to about 60 percent niobium, from about 30 percent to about 40 percent zirconium, balance titanium, said alloys being characterized by good hot hardness properties.
3. Titanium-niobium-base alloys of the beta-phase type consisting of from about 30 percent to about 70 percent niobium, from about 30 percent to about 40 percent of an element from the group consisting of vanadium, zirconium, and tantalum, balance titanium.

#### References Cited in the file of this patent

#### UNITED STATES PATENTS

- 50 2,754,204 Jaffee et al. .... July 10, 1956  
 2,797,996 Jaffee et al. .... July 2, 1957  
 2,822,268 Hix .... Feb. 4, 1958

#### FOREIGN PATENTS

- 55 718,822 Germany .... Mar. 24, 1942  
 782,564 Great Britain .... Sept. 11, 1957

U

UNITED STATES PATENT OFFICE  
CERTIFICATE OF CORRECTION

Patent No. 3,038,798

June 12, 1962

Lewis W. Berger et al.

It is hereby certified that error appears in the above numbered patent requiring correction and that the said Letters Patent should read as corrected below.

Column 3, Table II, column 4, line 1 thereof, for "239" read -- 230 --; columns 3 and 4, Table III, column 4, line 14 thereof, for "780,000" read -- 78,000 --.

Signed and sealed this 16th day of October 1962.

(SEAL)

Attest:

ERNEST W. SWIDER  
Attesting Officer

DAVID L. LADD  
Commissioner of Patents